

## UNITED STATES PATENT OFFICE

2,311,772

ANTISEIZE LUBRICATING COMPOUND FOR  
THREADS AND ITS METHOD OF PREPARA-  
TION

Arthur L. Parker, Cleveland, Ohio

No Drawing. Application March 26, 1941,  
Serial No. 385,335

4 Claims. (Cl. 252—37)

This invention is concerned with a composition in the form of a thick paste or semi-solid for employment on threads and other parts formed of metals such as aluminum, aluminum alloy, etc., for service under conditions where there may be contact with water, air and natural gas.

A preferred composition comprises the following ingredients:

Mineral oil 16 gallons (120 pounds)  
Fused lead stearate 28 pounds

The preferred mineral oil is a paraffine type oil having a viscosity of 140 to 220 seconds by Saybolt's universal viscosimeter at 210 degrees F.; and having a flash point of 490 degrees F. and a fire point of 540 degrees F. Oils of a substantially less viscosity do not provide a product having the desired body, even in the presence of a larger quantity of stearate. Care should be taken to employ a neutral oil of high chemical stability for maximum advantage with threaded and like parts of aluminum or aluminum alloy.

The fused lead stearate is a metallic soap employed for giving, when properly compounded with the oil, better anti-seize properties than powdered stearates of lead, zinc or aluminum, and as being easier to incorporate with the oil than such powdered stearates. The fused lead stearate is preferred over aluminum stearate, as the latter undergoes decomposition during fusion; and is preferred over fused zinc stearate because zinc stearate undergoes a partial decomposition during fusion, and the fused product does not blend into the oil in a satisfactory manner for forming a stable product. The lead stearate is preferred over lead oleate since the latter has too low a melting point and is susceptible to oxidation; and likewise is preferred to lead palmitate which has a somewhat lower melting point than the stearate and does not lead to the stiff composition which is presently preferred. It will be understood, however, that lead palmitate and even a minor proportion of lead oleate may be tolerated in the material and at times employed where it is desired to have a particular physical consistency or viscosity with a relatively high percentage of the anti-seize ingredient or metallic soap, compared with the quantity of oil utilized.

In the above preferred composition, the ratio by weight is 81 per cent of oil to 19 per cent of stearate. It is, however, feasible to employ other proportions in which the stearate is present on the basis of 20 to 35 pounds per 120 pounds of oil, or roughly 13 to 23 per cent.

The lead stearate is a neutral material preferably prepared by fusing molecularly equivalent quantities of stearic acid and (bivalent) lead oxide until chemical union occurs, and a fused product is obtained. This product is then cooled and ground until the bulk is around 40 mesh, with the exclusion of particles in excess of 20 mesh, in order to present the stearate in such a finely divided form that it is quickly taken up by the oil during the blending operation. Obviously, a finer grind is feasible, at a relatively greater expense.

The composition is most advantageously formed by heating the oil to a temperature of at least 130 degrees C., and preferably not exceeding 160 degrees C. A suitable container such as an agitated grease kettle or a kettle having mechanical mixing device, can be employed for the operation. The ground particles of the fused lead stearate are then introduced slowly with constant agitation, and with maintenance of the temperature. As the particles of fused stearate come into contact with the oil, they are melted and then blended into the oil. It has been found that when a lesser temperature than 130 degrees C. is utilized, or when large quantities of stearate are suddenly introduced, the oil forms an initial coating around a particle or a group of particles of the stearate and that therewith a ball of unmelted stearate is maintained in spite of a lengthy agitation or considerable increase of temperature, as the coating of oil appears to act as an insulator to prevent the blending. It has, however, been found possible also to intermingle the stearate by slowly mixing with the oil at substantially room temperature, and then bring the entire mass to a temperature in excess of 130 degrees and by continuously agitating produce a composition of uniform nature; but this method leads to foaming and sometimes to a lumping which cannot be dissipated without heating to a relatively higher temperature than employed with the preferred procedure.

The blending operation may be followed by observing the appearance as to freedom from small lumps or particles of unmelted stearate which are readily visible even into the later stages of blending. When the contents of the kettle appear to have a uniform consistency, a spatula or test stick is dipped into the mixture and withdrawn. As the composition cools, a coating forms on the spatula, and can be rubbed between the fingers: if found free of lumps and smooth and uniform, the blending is satisfactorily completed, while if there is an appearance

or "touch" of graininess, or the presence of small particles is observed, heating and stirring is continued until the desired smooth and uniform product is obtained.

The contents of the mixing vessel are then cooled to about 100 degrees C., and packaged in cans or other suitable containers.

The preferred final product has a A. S. T. M. penetration reading of 240 to 300 at room temperature (72 degrees F.), and a negative response as to corrosion of metal.

The material is employed by applying sparingly and evenly to the threaded or other parts before assembly.

It is obvious that the invention is not limited solely to the ingredients and proportions described, but may be employed in modified form within the scope of the appended claims.

I claim:

1. An anti-seize paste for sealing threaded joints and like parts between metals, comprising a mineral oil having a viscosity of at least 140 seconds Saybolt at 210 degrees F., and fused lead stearate intimately blended with the oil, the oil and stearate being present substantially in the proportion by weight of 120 parts of oil for 20 to 35 parts of stearate.

2. An anti-seize paste for sealing threaded joints and like parts between metals, comprising a mineral oil of paraffine type having a viscosity of 140 to 220 seconds Saybolt at 210 degrees F. with a flash point of substantially 490 degrees

F. and a fire point of substantially 540 degrees F., together with fused lead stearate intimately distributed in said oil to provide a smooth and uniform paste, the oil and stearate being present substantially in the proportion by weight of 120 parts of oil for 28 parts of the stearate, the paste having an A. S. T. M. penetration reading substantially between 240 and 300 at room temperature.

10 3. The method of forming an anti-seize paste for sealing threaded joints and like parts, which comprises heating a mineral oil of paraffine type having a viscosity of 140 to 220 seconds Saybolt at 210 degrees F. to a temperature of 130 to 160 degrees C., bringing finely divided fused lead stearate in successive small quantities into the hot oil, stirring throughout the addition of stearate and until the mass is of smooth uniform consistency, the stearate being added until the proportion by weight is substantially 120 parts of oil for 20 to 35 parts of stearate, and then cooling.

4. An anti-seize paste for sealing threaded joints and like parts comprising a stable non-corrosive base consisting of a neutral mineral oil of paraffine type having a viscosity of at least 140 seconds Saybolt at 210 degrees F., and neutral fused lead stearate intimately blended with the oil, substantially in the proportions of 120 parts by weight of mineral oil to 28 parts by 30 weight of fused lead stearate.

ARTHUR L. PARKER.